

1

2,827,357

**CONTINUOUS DYEING OF VEGETABLE FIBRES  
WITH VAT DYES**

Robert S. E. Hannay, Darnick, Melrose, and William Kilby, Eden Park, Lancaster, England, assignors to Standfast Dyers & Printers Limited

No Drawing. Application April 4, 1955  
Serial No. 499,243

Claims priority, application Great Britain April 8, 1954

9 Claims. (Cl. 8—34)

This invention relates to the continuous dyeing with vat dyes of cotton, linen or other vegetable fibres which latter term is to be taken as embracing the fibres whether in the form of fabrics, yarns, filaments or the like.

The term "continuous dyeing" is intended to refer to that class of dyeing in which the material to be dyed is continuously passed into, through, and out of an aqueous dyebath, as distinct from batch dyeing in which the material is dyed in batches which are intermittently inserted and taken out of the dyebath.

It has been known to dye yarns or fabrics continuously with vat dyes, using aqueous dye liquors containing caustic alkali and sodium hydrosulphite. The alkali strength of such dye liquors is determined by the quantity of dyestuff and hydrosulphite used, but does not normally exceed 60 grammes per litre.

We have found as a result of experiment that considerable economy in dyestuff cost can be attained in said continuous dyeing processes if the concentration of caustic alkali in the aqueous vat dye liquor is increased to a marked degree.

In accordance with the invention we provide a process for continuous dyeing of vegetable fibrous material with vat dyes characterised by the step of passing the material continuously through an aqueous dyebath in which there is a caustic alkali concentration of between approximately 120 (one hundred and twenty) grammes per litre and 400 (four hundred) grammes per litre.

A preferred concentration is of the order of 200 (two hundred) grammes per litre, and it has been found that this leads to a fifty percent reduction in dyestuff costs with some dyestuffs. Thus the total consumption of dye utilising the process according to the invention is much less for a given quantity of material and the same shade, than with the hitherto normal method of dyeing, as a given amount of dyestuff gives a greater colour value in the relatively short time available in a continuous dyeing process. Thus material dyed by the hitherto normal process will contain considerably more dyestuff than the same material dyed to the same shade under the process of the invention.

The strength of the caustic alkali may be varied with different vegetable fibres, while caustic soda may be used or may be wholly or partly replaced by caustic potash, sodium zincate, or other alkaline substances known to have a swelling action on cellulose fibres.

Vat dyestuffs which have been found suitable for the process include inter alia:

Caledon Yellow GNS (I. C. I.) (C. I. 1118)-Flavanthrone,  
Caledon Direct Black G. S. (I. C. I.).  
Caledon Gold Orange 3GS (I. C. I.).  
Caledon Red BNS (I. C. I.) (C. I. 1162) 1, 2 anthraquinonenaphthacridone.  
Paradone Bordeaux RR (L. B. Holliday).  
Caledon Olive Green BS (I. C. I.).  
Caledon Green 7GS (I. C. I.).

2

Caledon Oliver RS (I. C. I.) (C. I. 1150)—obtained by treating 4:4'-dibenzoylamino-1:1' dianthrimide with sulphuric acid.

5 Caledon Brown RS (I. C. I.) (C. I. 1151)—obtained by treating 4:5 dibenzoylamino-1:1' dianthrimide with sulphuric acid.

Caledon Dark Brown 6RS (I. C. I.).

10 Caledon Brown GS (I. C. I.) (C. I. 1152)—a mixture of Caledon Olive RS and Caledon Brown RS above.

10 Caledon Brown BS (I. C. I.) (C. I. 1120).

Caledon Brill. Violet RS (I. C. I.) (C. I. 1135).

Caledon Yellow Brown 3GS (I. C. I.).

A continuous process may advantageously be used in accordance with our British Patents 620,584, 661,086,

15 681,983, 665,454 and 663,066, which utilise hot molten metal to apply heat and squeezing action on textile material during its continuous passage therethrough. Other continuous vat dyeing processes may, of course, be utilised in some of which steam or hot oil may replace the molten metal as the dye-fixing medium.

The following specific examples are now referred to:

*Example 1*

Dry, unscoured 4<sup>s</sup> Condenser cotton yarn in tape form 25 is heated to a temperature of 79° to 80° C. by passing over steam heated cylinders and is then passed into an aqueous dye liquor of small volume which floats on the surface of a molten metal bath and which has the following composition:

30 120 grms. per litre Caledon Dark Brown 6RS (Imperial Chemical Industries).

15 grms. per litre Caledon Yellow GNS-Flavanthrone (Imperial Chemical Industries) (Colour Index 1118).

35 20 grms. per litre Caledon Direct Black GS (Imperial Chemical Industries).

200 grms. per litre Caustic Soda.

31 grms. per litre Sodium Hydrosulphite.

15 grms. per litre Glucose Syrup.

40 20 grms. per litre Alcopol T (Allied Colloids) (Wetting and dispersing agent).

30 10 grms. per litre Dilford Special (Wetting agent) (Dilford Products).

45 The yarn passes continuously through the aqueous dye liquor and through the molten metal bath at a speed of 20 yards per minute giving an immersion time of 0.96 second for the dye liquor and 10.4 seconds for the molten metal. The molten metal is an alloy of Bismuth, Lead, Tin and Cadmium, with a melting point of 71° C., and is 50 maintained at 95° C. The aqueous dye liquor is made up and stored at room temperature and is pumped to the surface of the molten metal through a heater which raises the temperature to 75° C. The volume of dye liquor floating on the surface of the metal is automatically maintained constant.

55 The yarn leaves the molten metal through a 10% solution of Glauber's salt which floats on the exit surface and has a temperature of 90° C., and then passes through the common form of continuous after treatment range where it is oxidised, soaped and rinsed in known manner. The yarn so treated is coloured a nigger brown and is very considerably darker than yarn dyed in a hitherto normal dyebath which in this example would contain 24 grms. of caustic soda per litre.

60

*Example 2*

Dry, unscoured, 2/32<sup>s</sup> cotton yarn in tape form is dyed in the manner described in Example 1 but using the following aqueous dye liquor:

70 100 grms. per litre Caledon Red BNS—1,2 anthraquinone-naphthacridone (Colcur Index 1162).

200 grms. per litre Caustic Soda.

- 20 grms. per litre Sodium Hydrosulphite.  
 10 grms. per litre Glucose Syrup.  
 20 grms. per litre Alcopol T.  
 10 grms. per litre Dilford Special.

The red coloured yarn which results is about 50% darker than that resulting from the use of hitherto normal quantities of caustic soda which in this example would be 15 grms. per litre.

*Example 3*

Dry, scoured cotton drill fabric is dyed in a manner similar to the yarn of Example 1 but the fabric speed is 40 yards per minute and the aqueous dye liquor has the following composition:

- 100 grms. per litre Caledon Gold Orange 3 GS (Imperial Chemical Industries) (Colour Index).  
 200 grms. per litre Caustic Soda.  
 20 grms. per litre Sodium Hydrosulphite.  
 10 grms. per litre Glucose Syrup.  
 20 grms. per litre Alcopol T.  
 10 grms. per litre Dilford Special.

The resultant gold coloured fabric is about 25% darker than a similar dyeing using 15 grms. caustic soda per litre, which is the hitherto normal quantity.

*Example 4*

Dry, scoured, cotton drill fabric is dyed in a similar manner to Example 3, but using the following aqueous dye liquor:

- 100 grms. per litre Caledon Brown RS (C. I. 1151).  
 200 grms. per litre Caustic Soda.  
 20 grms. per litre Sodium Hydrosulphite.  
 10 grms. per litre Glucose Syrup.  
 10 grms. per litre Saponified Castor Oil (wetting agent).

*Example 5*

The process of Example 4 is repeated but the 200 grms. per litre caustic soda is replaced by 400 grms. per litre caustic potash.

*Example 6*

- 100 grms. per litre Caledon Red BNS (C. I. 1162).  
 5 grms. per litre Saponified Castor Oil (wetting agent).  
 20 grms. per litre Sodium Hydrosulphite.  
 10 grms. per litre Glucose Syrup.  
 15 grms. per litre Caustic Soda.

The above materials are added to 600 ccs. water at 20° C., and then there is added 22 grms. zinc oxide dissolved in 400 ccs. water containing 185 grms. caustic soda. This liquor, containing sodium zincate, is pumped to the surface of the molten metal bath, through a heater as in Example 3, and a cotton fabric passed through this liquor is dyed a fast red colour which is about 50% darker than that obtained with a bath of normal alkalinity.

As aforesaid, the process is applicable to other vegetable fibres; for example, bleached linen fabric can, with advantage, be dyed by the method of Example 3.

We claim:

1. A process of molten metal bath dyeing of vegetable fibrous material with vat dyes, comprising continuously passing the fibrous material through hot aqueous dye liquor containing a vat dye and an alkali metal hydrosulfite floating on the surface of said bath, said aqueous dye liquor containing about 120 to 400 grams per liter of caustic alkali.
2. A process according to claim 1 wherein the alkali metal hydrosulfite is sodium hydrosulfite.
3. A process according to claim 1 wherein the caustic alkali concentration is about 200 grams per liter.
4. A process according to claim 1 in which the aqueous dye liquor contains sodium zincate.
5. A process according to claim 1 wherein the dye bath also contains glucose.
6. A process according to claim 1 wherein the caustic alkali comprises caustic soda.
7. A process according to claim 6 wherein the alkali metal hydrosulfite is sodium hydrosulfite and is present in an amount of 20 to 31 grams per liter.
8. A process according to claim 7 wherein the dye bath contains 10 to 15 grams per liter of glucose.
9. A process according to claim 8 wherein the caustic soda is present in an amount of about 200 grams per liter.

References Cited in the file of this patent

FOREIGN PATENTS

- 40 99,337 Germany Sept. 13, 1898

OTHER REFERENCES

- 45 Jour. Soc. Dyers & Col. for December 1951, pages 509-513.  
 Jour. Soc. Dyers & Col. for July 1952, pages 249-256.